

## UNITED STATES PATENT OFFICE

2,286,662

## COLOR PHOTOGRAPHY

Edith Weyde, Cologne-Riehl, and Erwin Trabert, Leverkusen-Wiesdorf, Germany, assignors, by mesne assignments, to General Aniline & Film Corporation, New York, N. Y., a corporation of Delaware

No Drawing. Application August 30, 1939, Serial No. 292,608. In Germany September 2, 1938

## 8 Claims. (Cl. 95—2)

Our present invention relates to an improvement in color photography.

In multi-layer material used for the production of color pictures by the process of color development there are used in the silver halide emulsions color formers which are fast to diffusion and between the silver halide emulsion layers filter layers which may consist for example of colloidal silver. For example between the upper blue-sensitive and the middle orthochromatic layers there may be a yellow filter containing colloidal silver. It has been found that in the limiting zone between the filter layer and the adjacent emulsion layers undesired color fog is produced.

Our invention has for one object to provide a process of avoiding or diminishing this color fog.

Another object of the invention is the provision of a process in which the color development is conducted in the presence of a substance which is more easily oxidized than is the coupling component constituted by the developer substance.

An additional object of the invention resides in the provision of a process in which this reducing agent which hinders the formation of the fog is added to the developer solution.

Yet another object of the invention is to provide a process in which this reducing agent is incorporated to the emulsion layers, to the filter layers or in other layers or backings.

A further object of the invention consists in the provision of a process in which this reducing agent is added to the emulsion before the layer is cast.

Other objects of our invention will be seen from the following disclosure.

Suitable reducing agents are, for example, hydroxylamine and its derivatives and organic hydrazine compounds, for example phenylhydrazine sulfonic acid or phenylhydrazine carboxylic acid.

As developing substance there may be used para-phenylenediamine and its derivatives containing substituents in the nucleus or in one or both amino groups or indeed both in the nucleus and in the amino group or groups; also para-aminophenols and their substitution products.

The filter layers comprising colloidal silver may be made for instance as described in French Patent No. 816,296. Besides the silver halide emulsion layers and filter layers other layers, for instance the antihalation layer (see for instance French Patent No. 840,563) may be used for the addition of the reducing agent. The multi-layer material for color photography which is to be used in the invention may contain in the layers

5 dyestuff formers fast to diffusion such as are described in: U. S. applications Serial No. 10,704, filed March 12, 1935, No. 111,250, filed November 11, 1936, No. 72,718, filed April 4, 1936, No. 174,350, filed November 13, 1937, No. 90,726, filed July 15, 1936, No. 94,340, filed August 5, 1936, No. 241,014, filed November 17, 1938, No. 126,842, filed February 20, 1937, No. 158,860, filed August 13, 1937, No. 159,518, filed August 17, 1937, No. 164,499, 10 filed September 18, 1937, No. 166,832, filed October 1, 1937, No. 171,705, filed October 29, 1937, No. 171,701, filed October 29, 1937, No. 175,285, filed November 18, 1937, No. 176,058, filed November 23, 1937, No. 191,952, filed February 23, 1938, No. 15,586, filed June 24, 1938, No. 220,502, filed July 21, 1938, No. 254,235, filed February 2, 1939, No. 265,601, filed April 1, 1939, No. 265,758, filed April 3, 1939, No. 265,759, filed April 3, 1939, No. 284,250, filed July 13, 1939, No. 284,257, filed July 13, 1939, 15 No. 284,258, filed July 13, 1939, U. S. Patents No. 2,156,821, dated May 2, 1939, No. 2,154,918, dated April 18, 1939, French Patent No. 844,928.

Developer solutions containing the reducing agent may be used also for other photographic materials in which the color picture is produced by color development since by addition of the reducing agent there is no ill effect produced on the action of the developer.

The following Examples 1, 2 and 3 are prescriptions of suitable developers:

## Example 1

|                               |       |      |
|-------------------------------|-------|------|
| Water                         | cc    | 1000 |
| Potassium carbonate           | grams | 50   |
| Diethyl-para-phenylenediamine | do    | 3    |
| Potassium bromide             | do    | 1    |
| Hydroxylamine hydrochloride   | do    | 5    |

## Example 2

|                               |       |      |
|-------------------------------|-------|------|
| Water                         | cc    | 1000 |
| Potassium carbonate           | grams | 50   |
| Diethyl-para-phenylenediamine | do    | 3    |
| Potassium bromide             | do    | 1    |
| Hydroxylamine hydrochloride   | do    | 5    |
| Sodium sulfite sicc.          | do    | 3    |

## Example 3

|                                 |       |      |
|---------------------------------|-------|------|
| Water                           | cc    | 1000 |
| Potassium carbonate             | grams | 50   |
| Diethyl-para-phenylenediamine   | do    | 3    |
| Potassium bromide               | do    | 1    |
| Phenylhydrazine-3-sulfonic-acid | do    | 5    |

## Example 4

To a photographic halide silver emulsion which contains a color former fast to diffusion there are

added per kilo of the emulsion 5 grams of para-phenylhydrazine sulfonic acid.

*Example 5*

An emulsion of the sparingly soluble lead salt 5 of para-phenylhydrazine carboxylic acid is made and then added to the colloidal silver solution which is to serve as a yellow filter.

We claim:

1. In a process of color developing a multi-layer material, the several emulsion layers containing color formers and located between two adjacent emulsion layers a yellow filter layer carrying colloidal silver, the improvement which comprises conducting the color development in the 10 presence of hydroxylamine.
2. In a process of color developing a multi-layer material, the several emulsion layers containing color formers and located between two adjacent emulsion layers a yellow filter layer carrying colloidal silver, the improvement which comprises conducting the color development in the presence of an organic hydrazine compound.
3. A multi-layer material for color development comprising silver halide emulsion layers 25 containing color formers between two adjacent emulsion layers a yellow filter carrying colloidal silver, at least one of said layers containing a reducing agent capable of being more easily oxidized than is the substance in the developer which couples to form the color and of preventing formation of color fog during development of said material.
4. A multi-layer material for color development comprising silver halide emulsion layers 30 containing color formers, at least one of said emulsion layers containing a reducing agent capable of being more easily oxidized than is the

substance in the developer which couples to form the color and of preventing formation of color fog during development of said material, between two adjacent emulsion layers a yellow filter carrying colloidal silver.

5. A multi-layer material for color development comprising silver halide emulsion layers containing color formers between two adjacent emulsion layers a yellow filter carrying colloidal silver, at least one of said filter layers containing a reducing agent capable of being more easily oxidized than is the substance in the developer which couples to form the color and of preventing formation of color fog during development of said material.

6. A multi-layer material for color development comprising silver halide emulsion layers containing color formers between two adjacent emulsion layers a yellow filter carrying colloidal silver, at least one of said layers containing hydroxylamine.

7. A multi-layer material for color development comprising silver halide emulsion layers containing color formers between two adjacent emulsion layers a yellow filter carrying colloidal silver, at least one of said layers containing an organic hydrazine compound.

8. In a process of color-developing a multi-layer material, the several emulsion layers containing color formers and located between two adjacent emulsion layers, a yellow filter layer carrying colloidal silver, the improvement which comprises conducting the color development in the presence of a reducing agent selected from the class consisting of hydroxyl amines and organic hydrazine compounds.

EDITH WEYDE,  
ERWIN TRABERT.